

Patented June 10, 1924.

1,496,978

# UNITED STATES PATENT OFFICE.

EDWIN CORNING, OF KENWOOD, AND PERCY A. E. ARMSTRONG, OF LOUDONVILLE,  
NEW YORK.

## ALLOY STEEL FOR METAL-CUTTING TOOLS.

No Drawing. Application filed October 29, 1920, Serial No. 420,432. Renewed October 6, 1923.

To all whom it may concern:

Be it known that we, EDWIN CORNING, a citizen of the United States, and a resident of Kenwood, county of Albany, and State of New York, and PERCY A. E. ARMSTRONG, a subject of the King of Great Britain, and a resident of Loudonville, county of Albany, and State of New York, have invented a new and useful Alloy Steel for Metal-Cutting Tools, of which the following is a specification.

Our invention relates to alloy steel for metal cutting tools, having properties generally intermediate between carbon steel and high speed steel.

For small metal cutting tools, such as drills, taps, reamers and the like, carbon steel answers sufficiently well, takes a keen cutting edge and produces smooth finished work, but is limited in its application, because under heat it softens and dulls rapidly.

High speed steel, which is commonly used for somewhat larger drills and similar tools which have to withstand greater heat, is not, of course, rapidly softened by frictional heat, but, in addition to its high price, has the objection that the work produced is not so smooth and well finished as can be obtained by sharp edge carbon steel tools, for example, and a subsequent separate finishing operation is usually required. For example, drilled holes require finish reaming to produce satisfactory work. Furthermore, in the case of taps, for example, the teeth of the tap are often injured by the high temperatures required for heat treatment of high speed steel.

According to the present invention, an alloy steel is produced which is inexpensive to make as it contains about 95% or more of iron, the alloying constituents forming only a comparatively small part of the steel. The steel of the present invention contains chromium, vanadium and molybdenum and also contains silicon considerably in excess of the usual silicon content of steel, silicon being present in our improved alloy steel preferably to the extent of about 1%. This steel is hard and strong, takes and holds a keen cutting edge which is not materially softened, so as to become dulled, up to a temperature of about 650° F., and when made into tools for cutting metal, such as drills, taps, reamers and the like, can be used for the production of smooth finished work, without the

necessity for separate finishing operations, and does not require heat treatment at such high temperatures as in the case of high speed steel, so that there is practically no tendency for any burning off of the tips of the teeth of taps and similar tools during heat treatment. This steel has other features of advantage as hereinafter stated.

A good typical composition for an alloy steel in accordance with the present invention is as follows:

|            | Per cent. |
|------------|-----------|
| Carbon     | 1.10      |
| Silicon    | 1         |
| Chromium   | 1         |
| Molybdenum | 1         |
| Vanadium   | .25       |
| Manganese  | .25       |

and the remainder iron. Tools made from material of this composition give surprisingly good results in use, it being found possible, for example, with twist drills made therefrom to drill many times the number of holes possible with ordinary twist drills, before the drill has to be resharpened.

Drills were made from steel substantially like the composition of the foregoing example, with the sole exception that the silicon was reduced to about .65%, and were found to give results but little improved over ordinary drills, thus evidencing the importance of a proper quantity of silicon in the composition.

More or less variation is possible without substantial detriment to the desirable qualities of the material and good results are obtained with varying quantities of the several components within substantially the following range:

|            | Per cent.    |
|------------|--------------|
| Carbon     | 1.05 to 1.20 |
| Silicon    | .85 to 1.10  |
| Molybdenum | .85 to 1.10  |
| Chromium   | .85 to 1.10  |
| Vanadium   | .15 to .30   |
| Manganese  | .20 to .50   |

The manganese can be dispensed with, if desired, and relatively small proportions of other materials commonly encountered in steel may, of course, be present.

Our improved alloy steel has a wide range of hardening temperatures. When heated to about 1500° F. and quenched in oil or water it has great hardness. When heated

2

to about 1850° F. and quenched the best results appear to be secured and a very excellent metal cutting steel is produced, with excellent strength and wear resisting properties and capacity to take and hold a very keen cutting edge. Such heating should preferably be performed in a quick heating medium, such as a molten salts bath. A very short time at such heat, preferably not 10 to exceed about one-half minute, is sufficient. This steel is one of the hardest steels which has been produced and when properly heat treated has a Brinell hardness of about 725-750. When drawn to 600° F., the Brinell hardness is still about 700. The steel works well in the mill, does not seam and can be cast into very smooth ingots. In rolling the temperature should not be carried unduly high and should preferably be kept under 2100° F. The steel will anneal and become quite easy to machine when properly annealed. There is very little tendency for this alloy combination to move, that is to say, to exhibit tendency to 20 warping, or other malformation upon heating up and quenching, which is a feature of great advantage in heat treatment of tools. The characteristic grinding spark given off in grinding articles made of our improved alloy steel, which does not contain tungsten, is markedly different from the tungsten colored spark. This is a feature of marked ad-

vantage both in manufacture and use, as this alloy steel can be readily distinguished from high speed steels by observation of the spark produced upon grinding. The foregoing applies whether the alloy steel is in the annealed or hardened state.

We claim:

1. As a new composition of matter, an alloy steel of analysis substantially as follows: carbon 1.10%, silicon 1%, chromium 1%, molybdenum 1%, vanadium .25%, manganese .25%, and the principal part of the remainder iron. 46
  2. As a new composition of matter, an alloy steel of analysis substantially as follows: carbon 1.05 to 1.20%, silicon .85 to 1.10%, molybdenum .85 to 1.10%, chromium .85 to 1.10%, vanadium .15 to .30%, manganese below .50%, and the principal part of the remainder iron. 50
  3. Metal cutting tools made from alloy steel as claimed in claim 1.
  4. Metal cutting tools made from alloy steel as claimed in claim 2. 55
  5. Drills for drilling metal made from alloy steel as claimed in claim 1.
  6. Drills for drilling metal made from alloy steel as claimed in claim 2. 60
- In witness whereof, we have signed our names hereto.
- EDWIN CORNING.  
PERCY A. E. ARMSTRONG.